

## 1

3,482,968

**TITANIUM BASE ALLOYS OF HIGH STRENGTH AT ATMOSPHERIC AND ELEVATED TEMPERATURES**  
Donald B. Hunter, Henderson, Nev., assignor to Titanium Metals Corporation of America, New York, N.Y., a corporation of Delaware  
No Drawing. Filed Aug. 8, 1967, Ser. No. 659,027  
Int. Cl. C22c 15/00

U.S. Cl. 75—175.5

7 Claims

### ABSTRACT OF THE DISCLOSURE

An age hardenable titanium base alloy consisting essentially of about 5-7% aluminum, 1-4% tin, 2-5% zirconium, 1-5% tungsten, up to 0.5% in total amount of carbon, oxygen and nitrogen, balance titanium apart from impurities within commercial tolerances, characterized by high strength and ductility at room and elevated temperatures and high creep strength at temperatures up to about 1100° F.

This invention relates to titanium base alloys which contain tungsten as an essential component, and which are characterized by high elevated temperature strength, thermal stress stability, good notch properties and good creep resistance. These properties are particularly desirable in the construction of modern high speed jet engine parts. The invention also relates to the processing of these alloys in a manner which serves to maximize their desired characteristics.

Titanium, because of its low density and high melting point is well adapted to high temperature structural applications in aircraft and the like. The pure metal alone, however, does not possess sufficient strength for most applications; and it must be alloyed with other metals in order to overcome this deficiency. Aluminum can be alloyed with titanium to provide increased strength; however the amount of aluminum must be kept below about 8% in order to preserve the ductility of the material. Tin, zirconium and molybdenum also add to the strength of

TABLE I.—ANALYSIS OF INGOTS

| Ingot No. | Nominal Composition       | Per-cent Al | Per-cent Sn | Per-cent Zr | Per-cent W | Per-cent O | Per-cent Fe | Per-cent N | Per-cent C | Per-cent Si | Density, lbs./cu. in. | Beta Transu  |
|-----------|---------------------------|-------------|-------------|-------------|------------|------------|-------------|------------|------------|-------------|-----------------------|--------------|
| V-3072    | Ti-6Al-2Sn-4Zr-2W         | 5.93        | 2.05        | 4.05        | 2.08       | 0.115      | 0.046       | 0.011      | 0.28       | .....       | 0.165                 | 11,875-1,900 |
| V-3428    | Ti-6Al-2Sn-4Zr-2W         | 5.98        | 1.98        | 3.82        | 2.03       | 0.130      | 0.062       | 0.007      | .....      | .....       | .....                 | .....        |
| V-3239    | Ti-6Al-2Sn-4Zr-4W         | 5.96        | 2.13        | 3.90        | 4.33       | 0.134      | 0.078       | 0.004      | .....      | .....       | .....                 | .....        |
| V-3418    | Ti-6Al-5Zr-1W-0.2Si       | 5.98        | .....       | 5.01        | 1.01       | 0.103      | 0.125       | 0.004      | .....      | 0.209       | 0.162                 | 21,875       |
| V-3001    | Ti-6Al-2Sn-4Zr-2Mo-0.25Si | 5.98        | 2.12        | 4.07        | 3 1.99     | 0.076      | 0.049       | 0.006      | .....      | 0.29        | .....                 | .....        |

<sup>1</sup> Accurate beta transus determination handicapped by segregation in ingot.

<sup>2</sup> Manufacturer's figure.

<sup>3</sup> Mo.

the material; and it has been found that a composition Ti-6Al-2Sn-4Zr-2Mo provides an excellent combination of strength, notch toughness and weldability. In order to achieve acceptable creep resistance in the temperature range of 1000-1100° F. however, there must be added an amount of silicon up to about 0.25%.

While the presence of silicon in a titanium base alloy serves to improve creep resistance, particularly at higher

temperatures, it does present other problems. The element silicon has a tendency to segregate during melting. Also, even small amounts of this element produce severe embrittlement of the titanium base alloy.

The present invention makes use of the discovery that silicon may be omitted entirely in titanium base alloys through the substitution of tungsten for molybdenum. It has been discovered that by virtue of this substitution, it becomes possible to fabricate a titanium base alloy which has high temperature creep resistance, strength and ductility.

The present invention makes possible the elimination of silicon in titanium base alloys without the attendant loss of creep resistance at high temperatures. Moreover, ductility and strength are preserved and have been found to be at least equal to any known titanium alloy. These advantages are achieved through the substitution of tungsten for molybdenum and the elimination of silicon.

It has further been discovered that by forging, rolling or subsequently annealing the metal above its beta transus temperature (i.e. above about 1885° F.), an exceptional combination of strength, creep resistance, notch toughness and thermal stability, not found in any presently available titanium base alloys, can be achieved.

The alloy of the present invention consists essentially of about 5 to 7% aluminum, 1 to 4% tin, 2 to 5% zirconium, 1 to 4% tungsten, up to 0.5% in total amount of carbon, oxygen and nitrogen, but preferably not to exceed 0.1% nitrogen and 0.2% carbon, balance titanium, apart from impurities within commercial tolerances.

A preferred alloy according to the invention is Ti-6Al-2Sn-4Zr-2W. Another preferred alloy is

### Ti-6Al-2Sn-4Zr-4W

For purposes of comparing properties of alloys according to the invention with closely related compositions containing silicon, compositions were melted in accordance with the following Table I, forged specimens of which were tested in various heat treated conditions and with results and as shown in the succeeding table hereof. Table I gives both the nominal and actual composition of the various alloys melted and tested.

Table II shows the room and elevated temperature tensile properties for the Ti-6Al-2Sn-4Zr-2W alloy in the various heat treated conditions shown. The heat treatments include sub-beta transus solution treatment followed by air cooling and aging. It will be observed that aged ultimate and 0.2% offset yield strengths up to 150-160K s.i. are obtained with excellent ductilities both as regards tensile elongation and area reduction values.

TABLE II.—ROOM AND ELEVATED TEMPERATURE TENSILE PROPERTIES OF Ti-6Al-2Sn-4Zr-2W<sup>1</sup>

| Ingot No. | Heat treatment                                                         | Test temp.,<br>° F. | UTS,<br>K p.s.i. | YS,<br>K p.s.i. | RA,<br>percent | Elong.,<br>percent | Modulus,<br>$E \times 10^{-6}$<br>p.s.i. |
|-----------|------------------------------------------------------------------------|---------------------|------------------|-----------------|----------------|--------------------|------------------------------------------|
| V-3428    | 1,575 F.-1 hr., AC                                                     | RT                  | 147              | 132             | 14.5           | 12                 | <sup>2</sup> 16.7                        |
| V-3428    | 1,575 F.-1 hr., AC                                                     | RT                  | 148              | 134             | 30             | 16                 | 16.6                                     |
| V-3428    | 1,675 F.-1 hr., AC                                                     | RT                  | 141              | 123             | 44             | 20                 | 15.7                                     |
| V-3428    | 1,675 F.-1 hr., AC                                                     | RT                  | 140              | 124             | 40             | 19                 | 16.4                                     |
| V-3428    | 1,775 F.-1 hr., AC                                                     | RT                  | 142              | 124             | 43             | 20                 | 16.1                                     |
| V-3428    | 1,775 F.-1 hr., AC                                                     | RT                  | 144              | 126             | 46.5           | 20                 | 16.4                                     |
| V-3428    | 1,825 F.-1 hr., AC                                                     | RT                  | 142              | 126             | 40             | 20                 | 16.5                                     |
| V-3428    | 1,825 F.-1 hr., AC                                                     | RT                  | 145              | 126             | 44             | 19                 | 16.5                                     |
| V-3428    | 1,675 F.-1 hr., AC plus 1,450 F.-15 mins., AC                          | RT                  | 139              | 124             | 29             | 17                 | 16.9                                     |
| V-3428    | 1,675 F.-1 hr., AC plus 1,450 F.-15 mins., AC                          | RT                  | 139              | 125             | 15             | 12                 | <sup>2</sup> 16.4                        |
| V-3428    | 1,675 F.-1 hr., AC plus 1,450 F.-15 mins., AC plus 1,100 F.-8 hrs., AC | RT                  | 145              | 131             | 15             | 13                 | 17.2                                     |
| V-3428    | 1,675 F.-1 hr., AC plus 1,450 F.-15 mins., AC plus 1,100 F.-8 hrs., AC | RT                  | 145              | 133             | 32             | 21                 | 17.0                                     |
| V-3428    | 1,825 F.-1 hr., AC plus 1,450 F.-15 mins., AC                          | RT                  | 141              | 128             | 28             | 17                 | 16.4                                     |
| V-3428    | 1,825 F.-1 hr., AC plus 1,450 F.-15 mins., AC                          | RT                  | 140              | 125             | 37             | 20                 | 16.3                                     |
| V-3428    | 1,825 F.-1 hr., AC plus 1,450 F.-15 mins., AC plus 1,100 F.-8 hrs., AC | RT                  | 146              | 139             | 17.5           | 15                 | <sup>2</sup> 17.1                        |
| V-3428    | 1,825 F.-1 hr., AC plus 1,450 F.-15 mins., AC plus 1,100 F.-8 hrs., AC | RT                  | 147              | 138             | 23             | 15                 | 17.2                                     |
| V-3428    | 1,575 F.-1 hr., AC plus 1,100 F.-8 hrs., AC                            | RT                  | 148              | 135             | 31             | 12                 | 16.2                                     |
| V-3428    | 1,575 F.-1 hr., AC plus 1,100 F.-8 hrs., AC                            | RT                  | 152              | 141             | 41             | 16                 | 16.6                                     |
| V-3072    | 1,675 F.-½ hr., AC plus 1,100 F.-8 hrs., AC                            | RT                  | 163              | 166             | 32             | 18                 | 16.4                                     |
| V-3072    | 1,675 F.-½ hr., AC plus 1,100 F.-8 hrs., AC                            | RT                  | 157              | 151             | 36             | 19                 | 16.4                                     |
| V-3072    | 1,775 F.-½ hr., AC plus 1,100 F.-8 hrs., AC                            | RT                  | 159              | 152             | 39             | 19                 | 16.0                                     |
| V-3072    | 1,775 F.-½ hr., AC plus 1,100 F.-8 hrs., AC                            | RT                  | 158              | 152             | 38             | 19                 | 16.0                                     |
| V-3072    | 1,825 F.-½ hr., AC plus 1,100 F.-8 hrs., AC                            | RT                  | 154              | 146             | 29             | 17                 | 17.6                                     |
| V-3072    | 1,825 F.-½ hr., AC plus 1,100 F.-8 hrs., AC                            | RT                  | 152              | 147             | 39             | 20                 | 16.1                                     |
| V-3428    | 1,875 F.-½ hr., AC plus 1,100 F.-8 hrs., AC                            | RT                  | 152              | 139             | 24             | 15                 | 16.6                                     |
| V-3428    | 1,875 F.-½ hr., AC plus 1,100 F.-8 hrs., AC                            | RT                  | 152              | 141             | 18             | 19                 | 16.5                                     |
| V-3072    | 1,625 F.-½ hr., AC plus 1,100 F.-8 hrs., AC                            | 800                 | 111              | 83              | 56             | 23                 | 12.0                                     |
| V-3072    | 1,625 F.-½ hr., AC plus 1,100 F.-8 hrs., AC                            | 900                 | 108              | 81              | 60             | 23                 | 11.7                                     |
| V-3072    | 1,625 F.-½ hr., AC plus 1,100 F.-8 hrs., AC                            | 1,000               | 95               | 75              | 62             | 23                 | 11.3                                     |
| V-3072    | 1,625 F.-½ hr., AC plus 1,100 F.-8 hrs., AC                            | 1,100               | 81               | 64              | 61             | 22                 | 9.7                                      |
| V-3072    | 1,775 F.-½ hr., AC plus 1,100 F.-8 hrs., AC                            | 800                 | 111              | 83              | 56             | 23                 | 12.5                                     |
| V-3072    | 1,775 F.-½ hr., AC plus 1,100 F.-8 hrs., AC                            | 900                 | 106              | 81              | 62             | 23                 | 12.8                                     |
| V-3072    | 1,775 F.-½ hr., AC plus 1,100 F.-8 hrs., AC                            | 1,000               | 96               | 76              | 58             | 22                 | 11.3                                     |
| V-3072    | 1,775 F.-½ hr., AC plus 1,100 F.-8 hrs., AC                            | 1,100               | 82               | 67              | 59             | 25                 | 9.8                                      |
| V-3072    | 1,825 F.-½ hr., AC plus 1,100 F.-8 hrs., AC                            | 600                 | 114              | 89              | 53             | 17                 | 12.9                                     |
| V-3072    | 1,825 F.-½ hr., AC plus 1,100 F.-8 hrs., AC                            | 800                 | 111              | 86              | 60             | 20                 | 11.6                                     |
| V-3072    | 1,825 F.-½ hr., AC plus 1,100 F.-8 hrs., AC                            | 900                 | 106              | 82              | 60             | 22                 | 10.9                                     |
| V-3072    | 1,825 F.-½ hr., AC plus 1,100 F.-8 hrs., AC                            | 1,000               | 97               | 78              | 62             | 24                 | 10.5                                     |
| V-3072    | 1,825 F.-½ hr., AC plus 1,100 F.-8 hrs., AC                            | 1,100               | 83               | 66              | 60             | 24                 | 10.1                                     |

<sup>1</sup> Processed below beta transus.<sup>2</sup> Flaw in specimen.

## Room temperature notch properties of

## Ti-6Al-2Sn-4Zr-2W

The following Table III shows the further enhancement <sup>40</sup> of aged strength for the alloy of Table II as similarly heat treated, except for quenching rather than air cooling from the solution treating temperature.

(i.e. Ingot No. V-3072)—notch time fracture, notch tensile and impact resistance—are given in Table IV below, following the various heat treatments shown.

TABLE III.—ROOM TEMPERATURE TENSILE PROPERTIES OF Ti-6Al-2Sn-4Zr-2W QUENCHED AFTER SOLUTION TREATMENT

| Ingot No.: | Heat treatment                             | UTS,<br>K p.s.i. | YS,<br>K p.s.i. | RA,<br>percent | Elong.,<br>percent | Modulus,<br>$E \times 10^{-6}$<br>p.s.i. |
|------------|--------------------------------------------|------------------|-----------------|----------------|--------------------|------------------------------------------|
| V-3072     | 1,650 F.-½ hr.-WQ                          | 148              | 126             | 45             | 20                 | 16.5                                     |
| V-3072     | 1,650 F.-½ hr.-WQ plus 900 F.-2 hrs.-AC    | 154              | 138             | 42             | 18                 | 18.4                                     |
| V-3072     | 1,650 F.-½ hr.-WQ plus 900 F.-4 hrs.-AC    | 156              | 143             | 42             | 18                 | 17.7                                     |
| V-3072     | 1,650 F.-½ hr.-WQ plus 900 F.-8 hrs.-AC    | 157              | 143             | 42             | 17                 | 16.4                                     |
| V-3072     | 1,650 F.-½ hr.-WQ plus 900 F.-16 hrs.-AC   | 152              | 140             | 42             | 17                 | 17.7                                     |
| V-3072     | 1,650 F.-½ hr.-WQ plus 1,050 F.-2 hrs.-AC  | 160              | 149             | 38             | 16                 | 16.8                                     |
| V-3072     | 1,650 F.-½ hr.-WQ plus 1,050 F.-4 hrs.-AC  | 162              | 149             | 35             | 16                 | 17.7                                     |
| V-3072     | 1,650 F.-½ hr.-WQ plus 1,050 F.-8 hrs.-AC  | 158              | 148             | 38             | 18                 | 16.1                                     |
| V-3072     | 1,650 F.-½ hr.-WQ plus 1,050 F.-16 hrs.-AC | 163              | 154             | 37             | 18                 | 19.6                                     |
| V-3072     | 1,650 F.-½ hr.-WQ plus 1,100 F.-2 hrs.-AC  | 162              | 151             | 39             | 18                 | 17.7                                     |
| V-3072     | 1,650 F.-½ hr.-WQ plus 1,100 F.-4 hrs.-AC  | 160              | 151             | 37             | 17                 | 16.5                                     |
| V-3072     | 1,650 F.-½ hr.-WQ plus 1,100 F.-8 hrs.-AC  | 161              | 151             | 35             | 18                 | 17.5                                     |
| V-3072     | 1,650 F.-½ hr.-WQ plus 1,100 F.-16 hrs.-AC | 158              | 148             | 35             | 17                 | 17.2                                     |
| V-3072     | 1,700 F.-½ hr.-WQ                          | 148              | 132             | 46             | 20                 | 16.8                                     |
| V-3072     | 1,700 F.-½ hr.-WQ plus 900 F.-2 hrs.-AC    | 154              | 140             | 45             | 17                 | 16.3                                     |
| V-3072     | 1,700 F.-½ hr.-WQ plus 900 F.-4 hrs.-AC    | 158              | 144             | 45             | 19                 | 16.6                                     |
| V-3072     | 1,700 F.-½ hr.-WQ plus 900 F.-8 hrs.-AC    | 160              | 147             | 41             | 17                 | 15.9                                     |
| V-3072     | 1,700 F.-½ hr.-WQ plus 900 F.-16 hrs.-AC   | 159              | 145             | 39             | 17                 | 17.2                                     |
| V-3072     | 1,700 F.-½ hr.-WQ plus 1,050 F.-2 hrs.-AC  | 164              | 152             | 41             | 17                 | 16.0                                     |
| V-3072     | 1,700 F.-½ hr.-WQ plus 1,050 F.-4 hrs.-AC  | 163              | 152             | 38             | 17                 | 16.8                                     |
| V-3072     | 1,700 F.-½ hr.-WQ plus 1,050 F.-8 hrs.-AC  | 166              | 153             | 35             | 17                 | 16.6                                     |
| V-3072     | 1,700 F.-½ hr.-WQ plus 1,050 F.-16 hrs.-AC | 160              | 148             | 36             | 17                 | 16.1                                     |
| V-3072     | 1,700 F.-½ hr.-WQ plus 1,100 F.-2 hrs.-AC  | 166              | 153             | 36             | 17                 | 17.5                                     |
| V-3072     | 1,700 F.-½ hr.-WQ plus 1,100 F.-4 hrs.-AC  | 163              | 153             | 36             | 17                 | 18.0                                     |
| V-3072     | 1,750 F.-1 hr.-WQ plus 900 F.-4 hrs.-AC    | 164              | 149             | 43             | 16                 | 16.3                                     |
| V-3072     | 1,750 F.-1 hr.-WQ plus 900 F.-8 hrs.-AC    | 164              | 148             | 43             | 17                 | 16.4                                     |
| V-3072     | 1,750 F.-1 hr.-WQ plus 1,050 F.-4 hrs.-AC  | 166              | 155             | 42             | 17                 | 15.2                                     |
| V-3072     | 1,750 F.-1 hr.-WQ plus 1,050 F.-8 hrs.-AC  | 167              | 156             | 40             | 14                 | 15.2                                     |
| V-3428     | 1,825 F.-1 hr.-WQ plus 1,100 F.-8 hrs.-AC  | 165              | 153             | 17             | 12                 | 16.1                                     |
| V-3428     | 1,825 F.-1 hr.-WQ plus 1,100 F.-8 hrs.-AC  | 163              | 153             | 16             | 10                 | 17.3                                     |
| V-3428     | 1,825 F.-1 hr.-WQ plus 1,100 F.-8 hrs.-AC  | 164              | 156             | 8              | 9                  | <sup>1</sup> 16.7                        |
| V-3428     | 1,825 F.-1 hr.-WQ plus 1,100 F.-8 hrs.-AC  | 164              | 152             | 14.5           | 12                 | 17.6                                     |

<sup>1</sup> Flaw in specimen.

TABLE IV.—ROOM TEMPERATURE NOTCH PROPERTIES OF Ti-6Al-2Sn-4Zr-2W<sup>1</sup>

| Heat treatment | Notch configuration,<br>$K_t$             | Notch time Fracture |                  | Notch tensile strength, K p.s.i. | Impact resistance, ft./lbs. |
|----------------|-------------------------------------------|---------------------|------------------|----------------------------------|-----------------------------|
|                |                                           | Passed, K p.s.i.    | Failed, K p.s.i. |                                  |                             |
| Ingots No.:    |                                           |                     |                  |                                  |                             |
| V-3072         | 1,675 F.-½ hr.-AC plus 1,100 F.-8 hrs.-AC | 2.8                 | 5 hrs. at 210    | 28 mins. at 220                  | 230 9.0                     |
| V-3072         | 1,675 F.-½ hr.-AC plus 1,100 F.-8 hrs.-AC | 2.8                 | do               | 27 mins. at 220                  | 233 9.25                    |
| V-3072         | 1,775 F.-½ hr.-AC plus 1,100 F.-8 hrs.-AC | 2.8                 | 5 hrs. at 220    | Broke loading at 230             | 238 9.5                     |
| V-3072         | 1,775 F.-½ hr.-AC plus 1,100 F.-8 hrs.-AC | 2.8                 | 5 hrs. at 200    | 4 hrs. 4 mins. at 210            | 237 12.5                    |
| V-3072         | 1,825 F.-½ hr.-AC plus 1,100 F.-8 hrs.-AC | 3.8                 | do               | 1 min. at 210                    | 225 -----                   |
| V-3072         | 1,825 F.-½ hr.-AC plus 1,100 F.-8 hrs.-AC | 3.8                 | do               | 4 mins. at 210                   | 221 -----                   |
| V-3072         | 1,825 F.-½ hr.-AC plus 1,100 F.-8 hrs.-AC | 8.2                 | 5 hrs. at 190    | Broke loading at 200             | 205 -----                   |
| V-3072         | 1,825 F.-½ hr.-AC plus 1,100 F.-8 hrs.-AC | 8.2                 | 5 hrs. at 180    | 12 mins. at 190                  | 203 -----                   |

<sup>1</sup> Processed below beta transus.

With a notch configuration of  $K_t=8$ , the alloy withstood at 5 hours at 180K p.s.i. Decreasing the severity of the notch to  $K_t=3.8$  enabled the alloy to withstand 5 hours at 200K p.s.i. With the sharper notch configuration of  $K_t=8$ , the notch tensile strength was over 200K p.s.i. while with a  $K_t=3.8$ , the notch tensile strength rose to 220K p.s.i.; and with a  $K_t=2.8$  the notch tensile strength rose to 230K p.s.i. Impact resistance was around 9 ft.-lbs. This compares with an impact resistance of 20–25 ft.-lbs. for Ti-6Al-2Sn-4Zr-2Mo with similar section sizes and heat treats.

The beta transus of Ti-6Al-2Sn-4Zr-2W is about 1885° F. NASA sharp notch properties of this alloy (i.e. Ingots No. 3428) after being processed and solution treated below the beta transus, are shown in Table V.

Table V demonstrates that the sharp notch values decrease with increase in aging time at 1100° F. On the other hand, Table V also shows that increasing the solution temperature tends to raise NASA sharp notch values for each aging time. Thus, with samples aged for 24 hours at 1100° F., increasing the solution temperature from 1675° F. to 1775° F., and then to 1825° F., raised the sharp notch values from 113 to 115, and then to 118. This demonstrates that employment of higher solution temperatures may be expected to improve the NASA sharp notch performance of Ti-6Al-2Sn-4Zr-2W.

The creep stability properties of Ti-6Al-2Sn-4Zr-2W (i.e. Ingots Nos. V-3072 and V-3428) processed and solution treated below the beta transus, are given in Table VI.

TABLE V.—NASA SHARP NOTCH PROPERTIES OF Ti-6Al-2Sn-4Zr-2W, V-3428, PROCESSED BELOW BETA TRANSUS AND AGED AT 1,100 F.

| Solution Treated at 1,675 F. |           |         | Solution Treated at 1,775 F. |           |         | Solution Treated at 1,825 F. |           |         |
|------------------------------|-----------|---------|------------------------------|-----------|---------|------------------------------|-----------|---------|
| Aging time, hours            | NASA, NTS | Average | Aging time, hours            | NASA, NTS | Average | Aging time, hours            | NASA, NTS | Average |
| 0                            | 140       | 137     | 0                            | 141       | 141     | 0                            | 135       | 142     |
|                              | 138       |         |                              | 140       |         |                              | 144       |         |
|                              | 134       |         |                              | 143       |         |                              | 146       |         |
| 2                            | 134       | 127     | 2                            | 116       | 123     | 2                            | 134       | 135     |
|                              | 124       |         |                              | 130       |         |                              | 134       |         |
|                              | 124       |         |                              | 124       |         |                              | 136       |         |
| 8                            | 127       | 119.5   | 8                            | 109       | 113     | 8                            | 125       | 124     |
|                              | 115       |         |                              | 111       |         |                              | 127       |         |
|                              | 119       |         |                              | 116       |         |                              | 120       |         |
|                              | 116       |         |                              | 107       |         |                              | 124       |         |
|                              | 121       |         |                              | 122       |         |                              | 125       |         |
| 24                           | 112       | 113     | 24                           | 115       | 115     | 24                           | 122       | 118     |
|                              | 120       |         |                              | 111       |         |                              | 113       |         |
|                              | 103       |         |                              | 119       |         |                              | 118       |         |
| 48                           | 107       | 106     | 48                           | 96        | 109     | 48                           | 106       | 112     |
|                              | 102       |         |                              | 115       |         |                              | 113       |         |
|                              | 109       |         |                              | 117       |         |                              | 117       |         |
| 96                           | 98        | 101.5   | 96                           | 106       | 102     | 96                           | 94        | 102     |
|                              | 104       |         |                              | 102       |         |                              | 114       |         |
|                              | 105       |         |                              | 94        |         |                              | 90        |         |
|                              | 99        |         |                              | 105       |         |                              | 110       |         |

TABLE VI.—CREEP STABILITY PROPERTIES OF Ti-6Al-2Sn-4Zr-2W<sup>1</sup>

| Ingots No. | Heat treatment                            | Creep Exposure |                  |             | Percent deformation | Subsequent Tensile Properties |              |             |                 |                                 |
|------------|-------------------------------------------|----------------|------------------|-------------|---------------------|-------------------------------|--------------|-------------|-----------------|---------------------------------|
|            |                                           | Temp., °F.     | Stress, K p.s.i. | Time, hours |                     | UTS, K p.s.i.                 | YS, K p.s.i. | RA, percent | Elong., percent | Modulus, $E \times 10^6$ p.s.i. |
| V-3072     | 1,675 F.-½ hr.-AC plus 1,100 F.-8 hrs.-AC | 800            | 70               | 150         | 0.091               | 159                           | 152          | 37          | 21              | 16.6                            |
| V-3072     | 1,675 F.-½ hr.-AC plus 1,100 F.-8 hrs.-AC | 1,000          | 30               | 150         | 0.194               | 157                           | 148          | 34          | 18              | 16.7                            |
| V-3072     | 1,675 F.-½ hr.-AC plus 1,100 F.-8 hrs.-AC | 1,000          | 30               | 150         | 0.373               | 157                           | 145          | 31          | 18              | 17.2                            |
| V-3072     | 1,675 F.-½ hr.-AC plus 1,100 F.-8 hrs.-AC | 1,100          | 15               | 150         | 0.924               | 155                           | 146          | 30          | 16              | 16.3                            |
| V-3072     | 1,675 F.-½ hr.-AC plus 1,100 F.-8 hrs.-AC | 1,100          | 15               | 150         | 2.303               | 161                           | 154          | 26          | 13              | 17.0                            |
| V-3072     | 1,675 F.-½ hr.-AC plus 1,100 F.-8 hrs.-AC | 1,100          | 15               | 150         | 1.386               | 161                           | 154          | 27          | 12              | 18.5                            |
| V-3072     | 1,675 F.-½ hr.-AC plus 1,100 F.-8 hrs.-AC | 1,100          | 18               | 150         | 0.416               | 159                           | 150          | 19          | 16              | 2 <sup>1</sup> 16.3             |
| V-3072     | 1,675 F.-½ hr.-AC plus 1,100 F.-8 hrs.-AC | 1,100          | 18               | 150         | 0.550               | 163                           | 150          | 24          | 16              | 2 <sup>1</sup> 17.2             |
| V-3072     | 1,650 F.-1 hr.-AC plus 1,100 F.-8 hrs.-AC | 1,100          | 15               | 150         | 0.957               | 155                           | 147          | 34          | 16              | 17.9                            |
| V-3072     | 1,650 F.-1 hr.-AC plus 1,100 F.-8 hrs.-AC | 1,100          | 15               | 150         | 1.261               | 155                           | 146          | 28          | 16              | 17.2                            |
| V-3072     | 1,650 F.-1 hr.-AC plus 1,100 F.-8 hrs.-AC | 1,100          | 18               | 150         | 1.902               | 155                           | 145          | 34          | 16              | 16.5                            |
| V-3072     | 1,650 F.-1 hr.-AC plus 1,100 F.-8 hrs.-AC | 1,100          | 18               | 150         | 1.199               | 154                           | 146          | 33          | 16              | 15.7                            |
| V-3072     | 1,775 F.-½ hr.-AC plus 1,100 F.-8 hrs.-AC | 800            | 70               | 150         | 0.133               | 153                           | 148          | 38          | 21              | 15.4                            |
| V-3072     | 1,775 F.-½ hr.-AC plus 1,100 F.-8 hrs.-AC | 1,000          | 30               | 150         | 0.290               | 160                           | 154          | 27          | 17              | 16.8                            |
| V-3072     | 1,775 F.-½ hr.-AC plus 1,100 F.-8 hrs.-AC | 1,000          | 30               | 150         | 0.278               | 158                           | 152          | 30          | 18              | 16.7                            |
| V-3072     | 1,775 F.-½ hr.-AC plus 1,100 F.-8 hrs.-AC | 1,100          | 15               | 150         | 0.177               | 157                           | 152          | 12          | 8               | 15.5                            |
| V-3072     | 1,775 F.-½ hr.-AC plus 1,100 F.-8 hrs.-AC | 1,100          | 18               | 150         | 0.814               | 170                           | 157          | 24          | 14              | 16.5                            |
| V-3072     | 1,825 F.-½ hr.-AC plus 1,100 F.-8 hrs.-AC | 800            | 70               | 150         | 0.117               | 152                           | 147          | 40          | 17              | 16.1                            |
| V-3072     | 1,825 F.-½ hr.-AC plus 1,100 F.-8 hrs.-AC | 800            | 70               | 150         | 0.095               | 154                           | 148          | 34          | 17              | 18.3                            |
| V-3072     | 1,825 F.-½ hr.-AC plus 1,100 F.-8 hrs.-AC | 900            | 50               | 150         | 0.220               | 156                           | 149          | 39          | 19              | 17.4                            |
| V-3072     | 1,825 F.-½ hr.-AC plus 1,100 F.-8 hrs.-AC | 900            | 50               | 150         | 0.213               | 152                           | 145          | 40          | 17              | 16.2                            |

See footnote at end of table.

TABLE VI.—CREEP STABILITY PROPERTIES OF Ti-6Al-2Sn-4Zr-2W<sup>1</sup>—Continued.

| Ingot No. | Heat treatment                            | Creep Exposure |                  |             | Percent deformation | Subsequent Tensile Properties |              |             |                 |                                    |
|-----------|-------------------------------------------|----------------|------------------|-------------|---------------------|-------------------------------|--------------|-------------|-----------------|------------------------------------|
|           |                                           | Temp., °F.     | Stress, K p.s.i. | Time, hours |                     | UTS, K p.s.i.                 | YS, K p.s.i. | RA, percent | Elong., percent | Modulus, $E \times 10^{-6}$ p.s.i. |
| V-3072    | 1,825 F.-½ hr.-AC plus 1,100 F.-8 hrs.-AC | 1,000          | 30               | 150         | 0.436               | 156                           | 148          | 32          | 17              | 15.3                               |
| V-3072    | 1,825 F.-½ hr.-AC plus 1,100 F.-8 hrs.-AC | 1,000          | 30               | 150         | 0.336               | 154                           | 147          | 36          | 19              | 19.2                               |
| V-3072    | 1,825 F.-½ hr.-AC plus 1,100 F.-8 hrs.-AC | 1,100          | 15               | 150         | 0.917               | 153                           | 144          | 34          | 17              | 14.9                               |
| V-3072    | 1,825 F.-½ hr.-AC plus 1,100 F.-8 hrs.-AC | 1,100          | 15               | 150         | 1.484               | 153                           | 144          | 31          | 18              | 16.1                               |
| V-3428    | 1,875 F.-½ hr.-AC plus 1,100 F.-8 hrs.-AC | 800            | 70               | 150         | 0.116               | 151                           | 143          | 15          | 12              | 17.1                               |
| V-3428    | 1,875 F.-½ hr.-AC plus 1,100 F.-8 hrs.-AC | 800            | 70               | 150         | 0.122               | 154                           | 146          | 35          | 19              | 18.5                               |
| V-3428    | 1,875 F.-½ hr.-AC plus 1,100 F.-8 hrs.-AC | 900            | 50               | 150         | 0.192               | 153                           | 143          | 31          | 19              | 18.1                               |
| V-3428    | 1,875 F.-½ hr.-AC plus 1,100 F.-8 hrs.-AC | 900            | 50               | 150         | 0.203               | 153                           | 144          | 25          | 16              | 17.1                               |
| V-3428    | 1,875 F.-½ hr.-AC plus 1,100 F.-8 hrs.-AC | 1,000          | 30               | 150         | 0.375               | 154                           | 147          | 28          | 16              | 17.4                               |
| V-3428    | 1,875 F.-½ hr.-AC plus 1,100 F.-8 hrs.-AC | 1,000          | 30               | 150         | 0.238               | 154                           | 146          | 18          | 14              | 16.3                               |
| V-3428    | 1,875 F.-½ hr.-AC plus 1,100 F.-8 hrs.-AC | 1,100          | 15               | 150         | 0.906               | 153                           | 145          | 6           | 13              | 19.4                               |
| V-3428    | 1,875 F.-½ hr.-AC plus 1,100 F.-8 hrs.-AC | 1,100          | 15               | 150         | 0.770               | 153                           | 144          | 12          | 7               | 18.1                               |

<sup>1</sup> Processed below beta transus.<sup>2</sup> Sample solution treated above 1,675 F. due to faulty furnace controller.<sup>3</sup> Flaw in specimen.<sup>4</sup> Broke on Vickers mark.

As shown in Table VI creep resistance is good. With 1000° F.-30K p.s.i.-150 hour exposures, creep deformations of 0.2-0.4% are found, which is similar to that of Ti-6Al-2Sn-4Zr-2Mo under the same conditions. The stability of Ti-6Al-2Sn-4Zr-2W after creep exposure is also good, with the sole exception of samples solution treated at 1875° F., close to the beta transus (estimated to be about 1890° F. in these samples), and exposed at 1100° F.

The alloy composition of the present invention exhibits remarkable mechanical properties when subjected to beta processing or beta annealing. The beta processing is achieved by rolling or forging the alloy at a temperature

above its beta transus (i.e. above about 1885° F.). Beta annealing is achieved by subjecting the alloy to a temperature above its beta transus (i.e. 1885° F.) for a period of about one half hour, air quenching to 1100° F. for about eight hours, and further air quenching to room temperature.

The important mechanical properties of Ti-6Al-2Sn-4Zr-2W (i.e. Ingots Nos. V-3072 and V-3428) beta annealed or beta processed, are given in Table VIII. The beta processed samples were subsequently solution treated below the beta transus at 1825° F., and all samples were aged for 8 hours at 1100° F.

TABLE VII.—MECHANICAL PROPERTIES OF BETA ANNEALED OR BETA PROCESSED T-6Al-2Sn-4Zr-2W

| Ingot No. | Heat treatment                       | Creep Exposure |                  |             | Percent deformation | Test temp., °F. | UTS, K p.s.i. | YS, K p.s.i. | RA, percent | Elong., percent | Modulus, $E \times 10^{-6}$ p.s.i. |
|-----------|--------------------------------------|----------------|------------------|-------------|---------------------|-----------------|---------------|--------------|-------------|-----------------|------------------------------------|
|           |                                      | Temp., °F.     | Stress, K p.s.i. | Time, hours |                     |                 |               |              |             |                 |                                    |
| V-3072    | 1,925 F.-½ hr.-AC+1,100 F.-8 hrs.-AC |                |                  |             |                     | RT              | 149           | 137          | 28          | 14              | 117.4                              |
| V-3072    | 1,925 F.-½ hr.-AC+1,100 F.-8 hrs.-AC |                |                  |             |                     | RT              | 157           | 146          | 21          | 14              | 118.3                              |
| V-3072    | 1,925 F.-½ hr.-AC+1,100 F.-8 hrs.-AC | 800            | 70               | 150         | 0.084               | RT              | 148           | 139          | 22          | 15              | 117.5                              |
| V-3072    | 1,925 F.-½ hr.-AC+1,100 F.-8 hrs.-AC | 800            | 70               | 150         | 0.100               | RT              | 149           | 141          | 22          | 15              | 118.0                              |
| V-3072    | 1,925 F.-½ hr.-AC+1,100 F.-8 hrs.-AC | 900            | 50               | 150         | 0.085               | RT              | 152           | 146          | 9           | 5               | 17.6                               |
| V-3072    | 1,925 F.-½ hr.-AC+1,100 F.-8 hrs.-AC | 900            | 50               | 150         | 0.071               | RT              | 150           | 142          | 8           | 3               | 17.3                               |
| V-3072    | 1,925 F.-½ hr.-AC+1,100 F.-8 hrs.-AC | 1,000          | 30               | 150         | 0.112               | RT              | 154           | 147          | 10          | 5               | 17.9                               |
| V-3072    | 1,925 F.-½ hr.-AC+1,100 F.-8 hrs.-AC | 1,000          | 30               | 150         | 0.117               | RT              | 151           | 144          | 8           | 5               | 16.9                               |
| V-3072    | 1,925 F.-½ hr.-AC+1,100 F.-8 hrs.-AC | 1,000          | 15               | 150         | 0.098               | RT              | 156           | 149          | 9           | 6               | 18.3                               |
| V-3072    | 1,925 F.-½ hr.-AC+1,100 F.-8 hrs.-AC | 1,000          | 15               | 150         | 0.132               | RT              | 152           | 144          | 10          | 6               | 17.9                               |

(B) Beta Processed

| Ingot No. | Heat Treatment                       | K <sub>t</sub> | Notch configuration          |                               | Notch Time Fracture |      |     | Impact resistance, ft. lbs. |
|-----------|--------------------------------------|----------------|------------------------------|-------------------------------|---------------------|------|-----|-----------------------------|
|           |                                      |                | Passed K <sub>t</sub> p.s.i. | Failed, K <sub>t</sub> p.s.i. | NTS                 | NTS  | NTS |                             |
| V-3072    | 1,825 F.-½ hr.-AC+1,100 F.-8 hrs.-AC | 3.8            | 5 hrs. at 200                | 1 hr. 31 mins. at 210         | 228                 | 13.0 |     |                             |
| V-3072    | 1,825 F.-½ hr.-AC+1,100 F.-8 hrs.-AC | 3.8            | .....                        | 4 mins. at 210                | 223                 |      |     |                             |
| V-3072    | 1,825 F.-½ hr.-AC+1,100 F.-8 hrs.-AC | 8.2            | 5 hrs. at 180                | 33 mins. at 190               | 208                 | 14.0 |     |                             |
| V-3072    | 1,825 F.-½ hr.-AC+1,100 F.-8 hrs.-AC | 8.2            | 5 hrs. at 190                | Broke loading at 200          | 204                 |      |     |                             |

<sup>1</sup> Samples below beta transus due to segregation.<sup>2</sup> Sample broke on knife edge, anomalous strengths recorded.<sup>3</sup> Sample broke in threads, possible flaw present.<sup>4</sup> Sample broke on Vickers mark.

As shown in Table VII for either beta annealing or beta processing the yield strengths are in the range of 135-150 K p.s.i. Also, the elastic modulus of the samples was increased by the beta treatment to the range of  $17.5 - 18.5 \times 10^6$  p.s.i.

The ductility of the beta processed samples was good, with the samples undergoing around 30% reduction in cross section area (RA).

exposure, the amount of deformation was also about 0.1%. Beta processed or beta annealed Ti-6Al-2Sn-4Zr-2W thus has a creep resistance similar to Ti-5Al-5Sn-5Zr over the entire temperature range of 800° F.-1100° F. This is the only alpha-beta alloy known to possess this quality.

Table VIII shows the results of increasing the tungsten content of the alloy of the present invention to a nominal value of 4% (i.e. Ingot No. V-3239).

TABLE VIII.—SOME PROPERTIES OF T-6Al-2Sn-4Zr-4W, V-3239

| Heat treatment                               | Creep Exposure  |            |                  | UTS, K p.s.i. | YS, K p.s.i. | RA, percent | Elong., percent | Modulus EX10 <sup>3</sup> p.s.i. |
|----------------------------------------------|-----------------|------------|------------------|---------------|--------------|-------------|-----------------|----------------------------------|
|                                              | Test temp., °F. | Temp., °F. | Stress, K p.s.i. |               |              |             |                 |                                  |
| 1,825 F.-30 mins.-AC plus 1,100 F.-8 hrs.-AC | RT              |            |                  | 162           | 149          | 27          | 16              | 17.4                             |
| 1,825 F.-30 mins.-AC plus 1,100 F.-8 hrs.-AC | RT              |            |                  | 167           | 154          | 25          | 16              | 17.6                             |
| 1,825 F.-30 mins.-AC plus 1,100 F.-8 hrs.-AC | 800             |            |                  | 122           | 94           | 59          | 21              | 13.1                             |
| 1,825 F.-30 mins.-AC plus 1,100 F.-8 hrs.-AC | 900             |            |                  | 116           | 91           | 65          | 21              | 12.2                             |
| 1,825 F.-30 mins.-AC plus 1,100 F.-8 hrs.-AC | 1,000           |            |                  | 107           | 86           | 66          | 20              | 12.8                             |
| 1,825 F.-30 mins.-AC plus 1,100 F.-8 hrs.-AC | 1,100           |            |                  | 98            | 78           | 71          | 19              | 10.5                             |
| 1,825 F.-30 mins.-AC plus 1,100 F.-8 hrs.-AC | RT              | 800        | 70               | 150           | 0.051        | 169         | 157             | 34                               |
| 1,825 F.-30 mins.-AC plus 1,100 F.-8 hrs.-AC | RT              | 1,000      | 30               | 150           | 0.188        | 169         | 162             | 6                                |
| 1,825 F.-30 mins.-AC plus 1,100 F.-8 hrs.-AC | RT              | 1,000      | 30               | 150           | 0.148        | 169         | 159             | 6                                |
| 1,825 F.-30 mins.-AC plus 1,100 F.-8 hrs.-AC | RT              | 1,100      | 15               | 150           | 0.110        | 168         | 160             | 6                                |
| 1,825 F.-30 mins.-AC plus 1,100 F.-8 hrs.-AC | RT              | 1,100      | 15               | 150           | 0.162        | 170         | 162             | 3                                |
| 1,725 F.-30 mins.-AC plus 1,100 F.-8 hrs.-AC | RT              |            |                  | 169           | 154          | 25          | 15              | 17.8                             |
| 1,725 F.-30 mins.-AC plus 1,100 F.-8 hrs.-AC | RT              |            |                  | 171           | 157          | 26          | 15              | 18.0                             |
| 1,725 F.-30 mins.-AC plus 1,100 F.-8 hrs.-AC | 800             |            |                  | 130           | 102          | 61          | 17              | 12.7                             |
| 1,725 F.-30 mins.-AC plus 1,100 F.-8 hrs.-AC | 1,100           |            |                  | 88            | 70           | 75          | 25              | 0.6                              |
| 1,725 F.-30 mins.-AC plus 1,100 F.-8 hrs.-AC | RT              | 1,000      | 30               | 150           | 0.389        | 177         | 169             | 5                                |
| 1,725 F.-30 mins.-AC plus 1,100 F.-8 hrs.-AC | RT              | 1,000      | 30               | 150           | 0.309        | 175         | 169             | 5                                |
| 1,825 F.-30 mins.-AC plus 1,200 F.-4 hrs.-AC | RT              |            |                  | 164           | 152          | 34          | 16              | 17.4                             |
| 1,825 F.-30 mins.-AC plus 1,200 F.-4 hrs.-AC | RT              |            |                  | 163           | 153          | 34          | 16              | 17.3                             |
| 1,825 F.-30 mins.-AC plus 1,200 F.-4 hrs.-AC | 800             |            |                  | 125           | 103          | 51          | 15              | 13.5                             |
| 1,825 F.-30 mins.-AC plus 1,200 F.-4 hrs.-AC | 1,000           |            |                  | 106           | 87           | 67          | 19              | 11.7                             |
| 1,825 F.-30 mins.-AC plus 1,200 F.-4 hrs.-AC | RT              | 1,050      | 30               | 24            | 0.267        | 169         | 160             | 6.5                              |
| 1,825 F.-30 mins.-AC plus 1,200 F.-4 hrs.-AC | RT              | 1,050      | 30               | 24            | 0.310        | 168         | 160             | 7.2                              |
| 1,825 F.-30 mins.-AC plus 1,200 F.-4 hrs.-AC | RT              | 1,050      | 30               | 24            | 0.209        | 168         | 160             | 7                                |

<sup>1</sup> Stress-strain curve not linear.

<sup>2</sup> Sample broke outside gage length.

<sup>3</sup> Sample broke on Vickers mark.

The elevated temperature yield strength of the samples of the invention was very good, being 83 K p.s.i. at 800° F. and 76 K p.s.i. at 1000° F. It was also found that the yield strength of the samples of the present invention, i.e. Ti-6-Al-2Sn-4Zr-2W consistently exceeded that of Ti-6Al-5Zr-1W-0.25Si.

The most noticeable improvement brought about by either beta annealing or beta processing Ti-6Al-2Sn-4Zr-2W was in the creep resistance shown as Table VII. In either condition, creep resistance was excellent, with deformations after a 1000° F.-30K p.s.i.-150 hour exposure being around 0.1%. With an 1100° F.-15K p.s.i.-150 hour

35 The results tabulated in Table VIII show that Ti-6Al-2Sn-4Zr-4W has even greater elevated temperature strength and creep resistance than Ti-6Al-2Sn-4Zr-2W although above 1000° F. it was somewhat more susceptible to creep embrittlement.

40 Table IX provides a comparison of the mechanical properties of beta processed Ti-6Al-2Sn-4Zr-2W (within the range of the present invention) and other alloys not within the range of the present invention but of the same general type (e.g. Ti-6Al-5Zr-1W-0.2Si and Ti-6Al-2Sn-4Zr-2Mo-0.25Si).

TABLE IX

[Comparison of Ti-6Al-2Sn-4Zr-2W, Ti-6Al-5Zr-1W-0.2Si and Ti-6Al-2Sn-4Zr-2Mo-0.25Si]

Processing methods:

Ti-6Al-2Sn-4Zr-2W: Beta process, Heat treated 1,825 F.-1/2 hr.-AC plus 1,100 F.-8 hrs.-AC.

Ti-6Al-5Zr-1W-0.2Si: Normal process, heat treated 1,910 F.-1 hr.-AC plus 930 F-24 hours.-AC.

Ti-6Al-2Sn-4Zr-2Mo-0.25Si: Beta process, heat treated 1,750 F.-1/2 hr.-AC plus 1,100 F.-8 hrs.-AC.

| Property                                                    | Ti-6Al-2Sn-4Zr-2W      | Ti-6Al-5Zr-1W-0.2Si    | Ti-6Al-2Sn-4Zr-2Mo-0.25Si |
|-------------------------------------------------------------|------------------------|------------------------|---------------------------|
| Density, lbs./cu. in.                                       | 0.165                  | 0.162                  | 0.163                     |
| RT 0.2% yield strength, K p.s.i.                            | 135-145                | 135-140                | 132                       |
| 800 F. 0.2% yield strength, K p.s.i.                        | 83                     | 75                     |                           |
| 1,000 F. 0.2% yield strength, K p.s.i.                      | 76                     | 71                     | 79                        |
| Notch tensile strength, K p.s.i., $K_t=8$                   | 206                    | 203                    |                           |
| Notch time fracture, K p.s.i., withstanding 5 hrs., $K_t=8$ | 180                    | 180                    |                           |
| Impact resistance, ft.-lbs.                                 | 13-14                  | 9-10                   |                           |
| NASA Sharp Notch Value:                                     |                        |                        |                           |
| Aged for 24 hours                                           | 110 (Aged at 1,100 F.) | 97 (Aged at 1,050 F.)  | 87 (Aged at 1,100 F.)     |
| Aged for 48 hours                                           | 102 (Aged at 1,100 F.) | 85 (Aged at 1,050 F.)  | 84 (Aged at 1,100 F.)     |
| Aged for 96 hours                                           | 104 (Aged at 1,100 F.) | 100 (Aged at 1,050 F.) | 71 (Aged at 1,100 F.)     |
| Creep Deformation with Exposures of:                        |                        |                        |                           |
| 850 F.-60 K p.s.i.-150 hours                                | 0.068%                 | 0.053%                 | <sup>2</sup> 0.104%       |
| 900 F.-50 K p.s.i.-150 hours                                | 0.080%                 | 0.090%                 | * 0.072%                  |
| 1,000 F.-30 K p.s.i.-150 hours                              | 0.103%                 | * 0.164%               | 0.108%                    |
| 1,100 F.-15 K p.s.i.-150 hours                              | 0.107%                 | 0.251%                 | 0.284%                    |

<sup>1</sup> Creep deformation figures are average of two, except for figures marked "\*" which are single values.

<sup>2</sup> 65 K p.s.i. load.

Table IX shows that at room temperature the 0.2% offset yield strength of the alloy of the present invention is somewhat greater than that of the silicon containing alloys. However, at increased temperatures, the alloy of the present invention exhibited much greater yield strengths than the silicon containing alloy which also contained tungsten; and while at the higher temperatures its yield strength was slightly below the other silicon containing alloy, its notch strength and creep resistance very greatly exceeded that of both silicon containing alloys.

The NASA Sharp Notch Values for the silicon free alloy of the present invention ranged between 110 and 102 when aged for different lengths of time at 1100° F. The NASA Sharp Notch Values for the silicon containing alloys, on the other hand, ranged between 71 and 100 for corresponding aging times and temperatures.

The creep resistance of the alloy of the present invention at elevated temperatures was far superior to the silicon containing alloys; and at 1100° F. the alloy of the present invention exhibited less than half the creep undergone by the silicon containing alloys under the same loads and durations.

It will be appreciated that the alloy of the present invention provides a combination of tensile strength, creep resistance, toughness and ductility at elevated temperatures which is unmatched by any other previously known alloy. Moreover, the improved mechanical properties of the alloy of the present invention are sharply enhanced when the alloy is either processed or annealed above its beta transus temperature.

What is claimed is:

1. An age hardenable titanium base alloy consisting essentially of about: 5-7% aluminum, 1-4% tin, 2-5% zirconium, 1-4% tungsten, up to 0.5% in total amount

10

15

20

25

30

35

of carbon, oxygen and nitrogen, balance titanium apart from impurities within commercial tolerances, characterized by high strength and ductility at room and elevated temperatures and high creep strength at elevated temperatures up to about 1100° F.

5 2. A titanium base alloy as in claim 1 wherein tungsten is present in the amount of about 2%.

3. A titanium base alloy as in claim 1 wherein tungsten is present in the amount of about 4%.

4. An age hardened alloy according to claim 1 having an ultimate strength of at least 150K p.s.i. and a tensile elongation of at least 10%.

5. An alloy according to claim 1 containing about 6% aluminum, 2% tin, 4% zirconium and 2 to 4% tungsten.

6. An alloy according to claim 1 containing about 6% aluminum, 2% tin, 4% zirconium and 2% tungsten.

7. An alloy according to claim 1 containing about 6% aluminum, 2% tin, 4% zirconium and 4% tungsten.

#### References Cited

##### UNITED STATES PATENTS

|           |         |                 |       |          |
|-----------|---------|-----------------|-------|----------|
| 2,769,707 | 11/1956 | Vordahl         | ----- | 75—175.5 |
| 3,049,425 | 8/1962  | Fentiman et al. | ----- | 75—175.5 |
| 3,105,759 | 10/1963 | Fentiman et al. | ----- | 75—175.5 |
| 3,378,368 | 4/1968  | Minton et al.   | ----- | 75—175.5 |

##### FOREIGN PATENTS

|         |        |                |
|---------|--------|----------------|
| 949,841 | 2/1964 | Great Britain. |
|---------|--------|----------------|

CHARLES N. LOVELL, Primary Examiner

U.S. Cl. X.R.

148—12.7, 32.5